

Patented Apr. 3, 1928.

1,664,675

# UNITED STATES PATENT OFFICE.

DAVID GESTETNER, OF LONDON, ENGLAND, ASSIGNOR TO D. GESTETNER LIMITED, OF LONDON, ENGLAND.

## DUPLICATING.

No Drawing. Application filed June 15, 1923, Serial No. 645,708, and in Great Britain October 27, 1922.

This invention relates to duplicating by the employment of flexible stencils comprising a foraminous support constituted by, for instance, yoshino or like paper and a stencil 5 layer formed of ink-resisting material, and has for its object to provide improvements in stencils of the character in question.

The invention consists in incorporating in the composition forming the stencil layer an 10 opaque pigment of a tint contrasting with the colour of the ink with which the stencil is to be used.

Ordinarily, the pigment will be an opaque white pigment.

15 Preferably, if the stencil layer is a gelatine or like composition a pigment is employed which has the effect, by itself or in combination with other constituents of the composition forming the stencil layer, of raising its 20 liquefying point and improving its qualities in other directions as, for instance, its resistance to the destructive action of the ink with which it is to be employed.

As examples of pigments which may be 25 employed, white zinc pigments or white titanium pigments may be mentioned. The use of the latter appears to be distinctly advantageous in the production of stencils produced by the action of light upon a gelatine 30 composition sensitized with bichromate, as it is found that this pigment assists in rendering the gelatine insoluble.

The employment of such pigments in combination with the wax-like compositions used 35 in forming so-called "wax stencils" is also of utility as it would seem that stencils containing pigments are less liable to be affected by climatic conditions. In this connection it may be remarked that the expression "wax-like composition" is intended to 40 include compositions which have the appearance of wax, as for instance compositions consisting wholly, mainly or in part of soaps.

One of the most obvious advantages of the 45 invention arises from the fact that when the stencil sheet is in use the matter which is to be reproduced by its employment is visible. In addition, defects can be observed in the stencil directly and not merely by observing the results of such defects in the duplicates produced by its employment.

50 The stencil sheet proper is (as is common in the art) conveniently secured to a detachable backing sheet, the whole being commonly referred to as a combined stencil sheet.

The purpose of the backing sheet is mainly to provide a substantially rigid or hard support for the sheet in cutting the stencil by means of a typewriter and the portion of the surface of the backing sheet corresponding 60 with the portion of the stencil sheet on which the stencil will be cut is in many cases black, being coated with printing ink with the object of rendering matter cut in the stencil more easily legible.

65 The object, however, is not sufficiently achieved in this way. If, however, the hard surfaced backing sheet is coated with a transferring ink over that portion of its surface which corresponds with the portion of the stencil sheet in which the impression is to be cut, the operation of cutting the stencil will cause an impression in the transferring ink to be produced on the stencil sheet wherever the stencil layer is cut and the matter cut in the stencil will then be clearly legible.

70 This, as will be recognized, is of great convenience and, for instance, reduces eye-strain on the part of the person cutting the stencil as well as in reading or checking it.

75 The transferring ink may be an ink similar to the oily or greasy inks used in duplicating; it may, for instance, be an ink comprising essentially a pigment suspended in mineral jelly. Alternatively, the ink may be similar in character to the wax and pigment compositions used in forming the so-called carbon paper.

80 The following particulars are given, by way of example, to illustrate suitable modes of carrying the invention, as applied to the production of stencil sheets for use in making stencils by cutting with a style or in a typewriter, into effect:

### Example I.

85 3½ parts of a white titanium oxide pigment such as a pigment containing titanium oxide and barium sulphate are added to 50 parts of a 20 per cent "solution" of gelatine to which also 15 parts of glycerine and 20 parts of water are added. Yoshino paper is 90 coated with this composition in known manner as, for instance, by drawing it over a roller partly immersed in the composition.

### Example II.

95 10 parts of a white titanium pigment are 100 added to 90 parts of a molten mixture con- 110

sisting of 40 parts of mutton tallow and 50 parts of paraffin wax of m. p. 135° F. and when the product is suitably mixed yoshino paper is coated with it in known manner.

5

*Example III.*

Sheets of a suitably hard-surfaced paper, such as has hitherto been used in forming the backing sheets of combined stencil sheets, 10 are provided over the greater portion of the surface of one side (the side which is to be next to the stencil, in cutting the same) with a coating of an ink formed by intimately mixing 8 parts of lamp-black with 15 100 parts of mineral jelly, by for instance a printing operation. To the sheet thus treated a stencil sheet formed in the manner described in either of the preceding examples

or in any other suitable manner is secured near one edge by means of an adhesive. 20

Having now described my invention what I claim as new and desire to secure by Letters Patent is:—

1. An improved flexible stencil sheet comprising a backing of yoshino or like paper 25 and covered with a stencil layer having in it a white titanium pigment.

2. An improved flexible stencil sheet having a foraminous support and covered with a stencil layer of a gelatine composition 30 having in it an insoluble pigment to assist in rendering the gelatine insoluble.

In testimony whereof I have signed my name to this specification.

DAVID GESTETNER.